

## UNITED STATES PATENT OFFICE

2,650,875

METHOD OF ETCHING ALUMINUM AND  
ALUMINUM BASE ALLOYS

Vladimir Dvorkovitz, Chicago, and John R. Swihart, Chicago Heights, Ill., assignors to The Diversey Corporation, a corporation of Illinois

No Drawing. Application December 9, 1950,  
Serial No. 200,117

11 Claims. (Cl. 41—42)

1

This invention relates to a method of etching aluminum and aluminum base alloys.

In many instances where articles of aluminum or aluminum base alloys are fabricated, it is necessary to etch the surface of the article either as an aid in fabrication of the article, to provide a base for further finishing or to give a final decorative finish. The usual industrial practice in etching the materials is to treat the surface of the article with a hot aqueous solution containing an etching alkali such as sodium hydroxide, potassium hydroxide, trisodium phosphate, soda ash or similar materials or mixtures of these chemicals in varying proportions. Because of the chemical activity of the aluminum, it reacts with these alkaline etching chemicals to form aluminum reaction products as may be represented by the reaction with sodium hydroxide:



Although such practices in the past have been effective in etching the metals, these methods are not entirely satisfactory and the method has certain inherent disadvantages. Probably the most important of these disadvantages is the formation of a hard rock-like scale or mass in the etching tank which is deposited on the sides of the tank, on the heating units in the tank and on other surfaces. This scale is ordinarily so hard and tenacious that it is quite difficult to remove. Generally this scale can only be removed by chipping it off with hammers or other tools. This not only causes loss of time and expensive labor costs but the breaking loose of the scale often damages the equipment. The scale is apparently formed when the concentration of the alkali in the etching solution becomes reduced due to the reaction of the alkali with the metal. When this happens the sodium aluminate reaction product reacts with water to precipitate aluminum hydroxide according to the equation:



The aluminum hydroxide apparently then reacts further to precipitate alumina according to the following equation:



The alumina is apparently the principal constituent of the hard rock-like scale.

2

It is known that the scale formation can be postponed for a short period by the addition of fresh alkali such as sodium hydroxide to the solution as the alkali in the solution is used up. However, as the concentration of aluminum in the solution increases, the addition of fresh alkali must be similarly increased in amount until these additions become so large that they upset the control necessary for the production of a uniformly etched product. Thus the attempt to solve the problem by additions of fresh alkali is not economically feasible.

As can be noted from the above equations, the reaction between the water and the sodium aluminate regenerates some sodium hydroxide. While this is of some advantage, it is more than counteracted by the objectionable scale that is also formed. Furthermore, this regeneration of alkali cannot be controlled so that as the work is withdrawn from the etching bath the regeneration often occurs in the film adhering to the work so that the increased concentration of alkali produces a non-uniform surface. Furthermore, the scale that is formed often adheres to the etched surface so that a high percentage of rejects are produced due to the difficulty of removal of this scale by subsequent treatment.

The following tabulated examples illustrate the rate at which this objectionable scale can form and the voluminous amounts of scale that are produced in comparison with the relatively small amount of caustic that is regenerated. The following results were obtained when an etching solution was aged and analyzed at various time intervals to determine the concentration of regenerated sodium hydroxide and scale. The results obtained were as follows:

| 40                                              | oz/gal.<br>of avail.<br>NaOH | oz/gal.<br>NaOH<br>regenerated | oz/gal.<br>Precipitate of<br>$\text{Al}_2\text{O}_3 \cdot 3\text{H}_2\text{O}$ |
|-------------------------------------------------|------------------------------|--------------------------------|--------------------------------------------------------------------------------|
| Fresh solution.....                             | 10.6                         | .....                          | 0.0                                                                            |
| Used solution.....                              | 1.2                          | 0.0                            | (1)                                                                            |
| Used solution, after $\frac{1}{2}$<br>hour..... | 3.0                          | 1.8                            | 7.1                                                                            |
| Used solution, after 8<br>hours.....            | 6.1                          | 4.9                            | 19.2                                                                           |

<sup>1</sup> Slight.

The above table of examples is only indicative of the results achieved since the degree of reversion is controlled by temperature, additions of

alkali as upkeep, the time of the etching process and other variables.

Applicants have successfully solved the problem of etching aluminum and aluminum base alloys without the formation of rock-like scale by employing a method wherein the article of aluminum or aluminum alloy is treated with a hot aqueous solution comprising an etching alkali and a small amount of a water soluble saturated aliphatic polyhydroxy inhibitor compound described in greater detail hereinafter. This new method operates either by preventing the reversion of the sodium aluminate to sodium hydroxide and alumina or by controlling this reversion so that any scale formed is in general granular and thus non-adherent to the surfaces contacted by the bath. In this latter instance the alumina precipitate forms as a sludge which can be easily washed away due to its non-adherent character.

The advantages of the new method of etching aluminum as described herein are numerous. Thus the invention prevents costly damage caused by the former necessity of cleaning the equipment by chipping the scale from this equipment. Furthermore, the operator of the etching bath can exercise better and closer control over the process so that the number of rejects are sharply reduced. The plant shutdowns necessary for repairs and to replace the spent etching solutions are kept to an absolute minimum. Also, the full benefit of the chemicals used in the new process is obtained as objectionable side reactions which tend to reduce the efficiency of the process are kept to a minimum. Other advantages are the improvement and uniformity in the quality of the work produced and the ease of disposal of the solid granular waste when the precipitate occurs. Furthermore, subsequent chemical treatments of the etched surfaces are often much easier than was true when prior etching processes were used. All of these improvements and advantages increase the economy, efficiency and ease of operation of the etching process.

The polyhydroxy inhibitors coming within the above described class include polyhydric alcohols having the formula  $\text{CH}_2\text{OH}(\text{CHOH})_a\text{CH}_2\text{OH}$ , wherein  $a$  is at least 1, starches having the general formula  $[\text{C}_6(\text{H}_2\text{O})_5]_x$ , sugars having the general formula  $\text{CHO}(\text{CHOH})_b\text{CH}_2\text{OH}$  wherein  $b$  is at least 3, polyhydroxy monobasic acids having the general formula  $\text{COOH}(\text{CHOH})_c\text{CH}_2\text{OH}$  wherein  $c$  is at least 4, polyhydroxy dibasic acids having the general formula



wherein  $d$  is at least 2, and acids having the generally formula  $\text{CHO}(\text{CHOH})_e\text{COOH}$  wherein  $e$  is at least 4. Among the preferred inhibitors are sorbitol as the polyhydric alcohol, corn starch, glucose and lactose as the sugars, gluconic acid as the monobasic acid and mucic acid as the dibasic acid. The salts or lactones of these substances may also be used. Similarly, gum arabic

as arabinose, rhamnose, galactose and fructose, which is a ketone sugar, starch and gum arabic are useful in controlling precipitation but sometimes excessive foaming occurs with these latter two materials. The most desirable inhibitors are gluconic acid, mucic acid, the alkali metal salts of these acids, glucoheptonic lactone, gluco lactone, corn starch, sorbitol and gum arabic. Gluconic acid or its salts appears to be the most desirable inhibitor because of its stability in heated solutions, uniformity of results obtained and commercial availability. If desired, the gluconic acid may be added as such to the etching solution where it is immediately converted to the alkali metal salt or the alkali metal salt itself may be added. This is, of course, true of any of the other acids. Glycerine and tartaric acid inhibit scale formation but are not preferred as their effectiveness is of short duration.

The mechanism by which these organic materials function to control the precipitation of alumina is not completely understood. However, the improved results of the new method have been proven in practical applications.

Several experiments were made using sodium gluconate in various amounts and as compared with a control employing sodium hydroxide and trisodium phosphate and a second control employing sodium hydroxide alone. In each test aluminum was etched at 180° F. in a solution containing 10 ounces per gallon of the etching chemicals. After no more aluminum would react with the solutions, these solutions were allowed to stand for eighteen hours after which they were examined for the effectiveness of the gluconate in preventing scale precipitation and adherence. The following results were obtained.

| Solution | 10 oz./gal. of Mix Containing—    | Percent    | Appearance of Precipitate | Adherence of Precipitate to Container |
|----------|-----------------------------------|------------|---------------------------|---------------------------------------|
| 1.....   | [NaOH]<br>[T. S. P.]              | 96<br>4    | Yes.....                  | Yes.                                  |
| 2.....   | NaOH                              | 100        | Yes.....                  | Yes.                                  |
| 3.....   | NaOH<br>Purified sodium gluconate | 95<br>5    | No.....                   |                                       |
| 4.....   | NaOH<br>Purified sodium gluconate | 98<br>2    | Yes.....                  | No.                                   |
| 5.....   | NaOH<br>Purified sodium gluconate | 99.5<br>.5 | Yes.....                  | Yes.                                  |

In order to control scale formation and utilize regenerated sodium hydroxide, two solutions were charged at 8 ounces per gallon in separate steel containers heated with steam coils at 160° F. Aluminum was dissolved for a period of 240 hours. This was equivalent to four times the theoretical amount which would react with the caustic present. At the end of that time, each container was examined for scale and precipitate. The following results were noted.

| Solution | 8 oz./gallon of Mix Containing—    | Percent | Amount of Precipitate        | Condition of Precipitate |
|----------|------------------------------------|---------|------------------------------|--------------------------|
| 1.....   | NaOH                               | 100     | Tank $\frac{2}{3}$ full..... | Hard rock-like mass.     |
| 2.....   | NaOH<br>Purified sodium gluconate. | 98<br>2 | Tank $\frac{1}{2}$ full..... | Sludge.                  |

which contains glucuronic acid from the family having the last previously described structural formula may also be used. Other sugars, such

The steam coils in solution 1 were coated with  $\frac{1}{2}$  inch of a hard white crystalline deposit which was removed only with difficulty. No solid resi-

due was observed on the cork used to heat solution 2.

A similar experiment using a mixture containing 97% sodium hydroxide and 3% technical sodium gluconate gave results similar to those obtained above with solution 2.

A further advantage obtained in using a suitable hydroxy compound as described herein is the elimination or the substantial reduction of the problems involved in removing smut often formed during aluminum etching. This smut is ordinarily silicon, carbon, copper or other materials left at the surface of the article being etched after removal of the aluminum by the etching solution. The removal of this smut often requires additional treatment in an acid bath. When aluminum and aluminum base alloys are treated according to the method of this invention the smut that remains can be removed much easier so that the removal time is reduced by  $\frac{1}{3}$  to  $\frac{1}{2}$  as compared with similar articles etched in a bath according to the old methods. In many instances, the new method leaves the smut in such a condition that it can be easily rinsed off so that the usual acid treatment is unnecessary.

In testing the methods of this invention it has been observed that crude and technical grades of gluconates and gluconic acid give somewhat better results than the purified material although the reason for this is not understood. The following data illustrates the differences in the crude or technical grade gluconate and the purified material.

| Solution | 10 oz./gal. of mix composed of—          | Percent    | Aluminum added                          | Precipitate Observed After—   |
|----------|------------------------------------------|------------|-----------------------------------------|-------------------------------|
| 1.....   | NaOH.....                                | 100        | Theoretical amount for caustic present. | 1 hour.                       |
| 2.....   | {NaOH.....<br>Purified sodium gluconate. | 95<br>5    | .....do.....                            | 45 hours.                     |
| 3.....   | {NaOH.....<br>Purified sodium gluconate. | 99.5<br>.5 | .....do.....                            | 18 hours.                     |
| 4.....   | {NaOH.....<br>Crude sodium gluconate.    | 99.5<br>.5 | .....do.....                            | 36 hours.                     |
| 5.....   | {NaOH.....<br>Crude sodium gluconate.    | 97<br>3    | .....do.....                            | None formed for<br>170 hours. |
| 6.....   | {NaOH.....<br>Tech. sodium gluconate.    | 97<br>3    | .....do.....                            | 96 hours.                     |

Similarly, it was discovered that as little as 0.1% of crude sodium gluconate by weight of the combined gluconate and sodium hydroxide would alter the character of the precipitate so that it was non-adherent.

Not all hydroxy organic compounds will produce the desired results in preventing or controlling the precipitate. In fact, certain hydroxy organic compounds appear to accelerate this scale formation. The following table illustrates the action on a comparative time basis of certain of these other materials.

| Material                                                     | Comparative Time of Scale Formation, Hours |
|--------------------------------------------------------------|--------------------------------------------|
| NaOH only, Control.....                                      | 0                                          |
| Itaconic acid.....                                           | -1/2                                       |
| Sorbic acid.....                                             | -1/2                                       |
| Aconitic acid.....                                           | -1/2                                       |
| 2,4 dimethylene gluconic acid.....                           | -1/2                                       |
| Lactic acid.....                                             | -1/2                                       |
| Citric acid.....                                             | +1/2                                       |
| Tetra sodium salt of ethylene diamine tetra acetic acid..... | -1/2                                       |
| Ethylene glycol.....                                         | -1/2                                       |

In contrast to this the materials used in the present methods produced the following comparative results:

| 5  | Material                    | Comparative Time of Scale Formation, Hours |
|----|-----------------------------|--------------------------------------------|
| 10 | NaOH only, control.....     | 0                                          |
|    | Glucoheptonic lactone.....  | +16                                        |
|    | Tartaric acid.....          | +2                                         |
|    | Malic acid.....             | +8                                         |
|    | U. S. P. gluconic acid..... | +16                                        |
|    | Corn starch.....            | +11                                        |
|    | Glucolactone.....           | +16                                        |
|    | Glucose.....                | +4                                         |
|    | Lactose.....                | +4                                         |
|    | Glycerine.....              | +1                                         |
|    | Sorbitol.....               | +16                                        |
|    | Gum arabic.....             | +16                                        |

A preferred composition for use in applicants' method is made up of 96% by weight of sodium hydroxide and 4% of technical 50% gluconic acid. This acid, of course, is converted immediately to sodium gluconate.

In the preferred method, the solution is maintained at a temperature of from 120° F. to 210° F. during the treatment and the polyhydroxy compound is present in an amount of 0.5% to 10% by weight of the combined alkali and the compound. In the preferred solutions the alkali is present in an amount of 4.0% to 10.0% by weight of the solution.

Having described our invention as related to the embodiments disclosed herein it is our inten-

tion that the invention be not limited by any of the details of description unless otherwise specified but rather be construed broadly within its spirit and scope as set out in accompanying claims.

We claim:

1. In the etching of articles of aluminum and of aluminum base alloys, the method which comprises treating the surface of said article with a hot aqueous solution comprising an etching alkali and a small amount of water-soluble saturated aliphatic polyhydroxy compound in a proportion such that the formation of a hard adherent precipitate is avoided for an extended period of time, said compound being selected from the class consisting of polyhydric alcohols of the formula  $\text{CH}_2\text{OH}(\text{CHOH})_a\text{CH}_2\text{OH}$  wherein  $a$  is at least 2, starches of the formula  $(\text{C}_6\text{H}_{10}\text{O}_5)_n$ , polyhydroxy monobasic acids of the formula



wherein  $c$  is at least 4, polyhydroxy dibasic acids of the formula  $\text{COOH}(\text{CHOH})_d\text{COOH}$  wherein  $d$  is at least 3, gum arabic and the alkali metal salts of said acids.

2. The method of claim 1 wherein said polyhydroxy compound is present in an amount of

0.1% to 20.0% by weight of the combined alkali and said compound.

3. The method of claim 1 wherein said solution is maintained at a temperature of 60° to 212° F. during said treatment.

4. The method of claim 1 wherein said polyhydroxy compound is present in an amount of 0.1% to 20.0% by weight of the combined alkali and said compound, the solution is maintained at a temperature of 60° to 212° F. during said treatment, and the alkali is present in an amount of 2.0% to 20.0% by weight of the solution.

5. The method of claim 4 wherein said alkali comprises sodium hydroxide and said polyhydroxy compound comprises sodium gluconate.

6. In the etching of articles of aluminum and of aluminum base alloys, the method which comprises treating the surface of said article with an aqueous solution containing 10 ounces per gallon of a mixture of 98% by weight of sodium hydroxide and 2% by weight of sodium gluconate

while maintaining said solution at a temperature of about 160° to 180° F.

7. The method of claim 1, wherein said aliphatic polyhydroxy compound is glucoheptonic lactone.

8. The method of claim 1, wherein said aliphatic polyhydroxy compound is gluconolactone.

9. The method of claim 1, wherein said aliphatic polyhydroxy compound is gluconic acid.

10. The method of claim 1, wherein said aliphatic polyhydroxy compound is mucic acid.

11. The method of claim 1, wherein said aliphatic polyhydroxy compound is sorbitol.

VLADIMIR DVORKOVITZ.  
JOHN R. SWIHART.

References Cited in the file of this patent

UNITED STATES PATENTS

|    | Number    | Name     | Date         |
|----|-----------|----------|--------------|
| 20 | 2,168,909 | Mason    | Aug. 8, 1939 |
|    | 2,318,559 | Percival | May 4, 1943  |